

Sept. 13, 1932.

A. O. AUSTIN

1,876,582

COATING AND HEAT TREATING

Original Filed May 25, 1923



INVENTOR  
Arthur O. Austin.  
BY *Alpheus J. Crane*  
ATTORNEY

## UNITED STATES PATENT OFFICE

ARTHUR O. AUSTIN, OF NEAR BARBERTON, OHIO, ASSIGNOR, BY MESNE ASSIGNMENTS,  
TO THE OHIO BRASS COMPANY, OF MANSFIELD, OHIO, A CORPORATION OF NEW  
JERSEY

## COATING AND HEAT TREATING

Original application filed May 25, 1925, Serial No. 32,709. Divided and this application filed September 14,  
1928. Serial No. 305,976.

This invention relates to a method and apparatus for coating and heat treating metal articles and has for its object the provision of a method and apparatus in which a uniform coating may be economically applied to the articles and in which difficulties that heretofore have been experienced are largely avoided.

The invention also, includes heat treatment of articles simultaneously with the coating operation. In the accompanying drawing there is illustrated apparatus by means in which the present invention may be performed. This apparatus together with the process comprised in the invention, is described in the following specification, the invention being more particularly pointed out in the appended claims.

In the drawing:  
20 The figure is a vertical sectional view showing one form of apparatus for practicing the present invention.

This application is a division of application, Serial Number 32,709, filed May 25, 25 1925.

This invention deals with new and improved methods of galvanizing and heat treating articles. In galvanizing, tinning or coating articles with lead or other material, it is generally desirable to form a uniform coat which amalgamates with the material covered and acts as a water protection.

While the invention applies particularly to galvanizing or the process of coating steel, grey iron and malleable castings with zinc, it applies to coating with some other metals such as tin. In the process of galvanizing, it is customary to clean the article by sand or shot blast or by pickling in acid. In the pickling operation, a coating may exist which acts as a flux so that when the article to be galvanized or tinned is placed in the bath, an amalgamation takes place. Where articles are simply clean and bright, it is generally necessary to dip the articles in a flux such as zinc chloride or sprinkle the articles with ammonium chloride commonly known as salammoniac. If the galvanizing or tinning bath is not very hot, an amalgamation usually takes place without much difficulty, provid-

ing the usual pains are taken. Where the amount of material galvanized is large, however, the bath is cooled. This makes it necessary to keep the articles to be galvanized or tinned in the bath long enough so that they can all become heated up, otherwise, if they are taken out of the bath they will have too thick a coat and there may be no amalgamation owing to the chilling of the coating material in contact with the pieces.

One method of correcting this difficulty is to run the molten bath at a higher temperature. This greatly speeds up the operation but in many cases it is open to serious difficulties. Where a bath of high temperature is used, there is a tendency to oxidize the surface of the article to be galvanized or tinned if amalgamation does not take place in a very short time such as may happen if there is a small amount of air or gas entrapped. This makes it exceedingly difficult to use a high temperature bath on many classes of ware which are galvanized or tinned. If the hot bath comes in contact on one side of the metal to be coated and an air or gas pocket exists on the opposite side of a thin section, the surface may become oxidized or the flux driven off so that amalgamation will not take place readily unless more flux is applied or considerable length of time is allowed. Where the surface becomes oxidized or the flux is driven off before amalgamation takes place, a bare spot or pinhole in the galvanizing or tinning usually results.

One object of the present invention is to get away from this difficulty. This is accomplished by placing the article to be coated in a molten bath which has a relatively low temperature. Where the bath is at low temperature, the tendency to drive off the flux before amalgamation takes place is not so great and the tendency to oxidize the surface is also reduced so that amalgamation takes place with a minimum amount of fluxing and without the formation of bare spots or pinholes. After amalgamation takes place, the surface of the article to be galvanized or tinned will not be affected by an increase in temperature and oxidization or the driving off of flux will not matter. The next step is

to transfer the articles galvanized to a bath which is much hotter. This is frequently quite important when a thin uniform coat is desired or where large production is desired. In order to insure uniformity, steps may be taken so that temperature is finally raised to the desired value. This can be readily done in one of several ways, depending upon the conditions.

10 One form of apparatus for accomplishing the desired results is shown in the drawing. In this case a tube 50 is filled with a molten bath and the articles 51 are put in at the charging end 52 and discharged at the end 53. The tubular member 50 containing the molten material may be of metal or a suitable refractory. The heating may be accomplished by any suitable fuel or by electrical energy as shown. Since the incoming material 20 enters the end 52, it will tend to lower the temperature of the bath at this point. As the material traverses toward the end 53 it will be heated up. This movement may be provided by magnetic apparatus in the case 25 that a refractory or non-magnetic tube is used or by a mechanical feeder 53' which periodically shoves the pieces 51 forward. If the heating turns are concentrated at the discharge end, a higher temperature will be 30 provided at that end which, with the cooling action at the entering end will tend to maintain a temperature difference with its advantages as previously explained. With this system an enclosed tube may be used which 35 will prevent the bath from coming into contact with the air or gases except at the entering and discharging ends, so that there will be little oxidation.

Where the refractory tube is used, the 40 amount of dross will be reduced to a minimum and under favorable conditions no dross will be formed. This is a very material advantage in that one of the principal objections to high temperature is the amount of dross 45 formed. As the piece is discharged from the end 53 it may be allowed to fall a considerable distance and strike several baffles 54 and 55 before falling into the quench tank 56. Striking several baffles tends to knock off 50 any superfluous material and if time sufficient is allowed before striking the cooling bath, the surface tension will tend to form a very uniform coat. Instead of striking baffles, it is possible to allow the article to fall 55 through a passage into which air is forced at a considerable velocity. This tends to blow off any superfluous material and the direction of the air may be used to retard the fall giving ample time to remove the superfluous material. With the methods shown, 60 it is possible to raise the material to the desired temperature so that the article may be tinned or galvanized and at the same time, give a heat treatment to increase the mechanical strength, hardness or reliability. 65

This method is applicable to the heating of articles for heat treatment as well as for the galvanizing or tinning operation.

I claim:

1. Apparatus for coating metal articles 70 comprising a container for a molten bath of coating material, means for heating the coating material in said container to higher temperatures at the point of exit of said articles than at the point of entrance, and means 75 for excluding air from the portion of said container most highly heated.

2. Apparatus for coating metal articles, 80 comprising a container of refractory material having a portion thereof closed at the top, means for feeding articles progressively through said container and electrical means for heating a bath of molten coating metal to different temperatures at different portions 85 of said container.

3. Galvanizing apparatus, comprising a tank having a covered portion and having an entrance opening at one side of said covered portion and an exit opening at the opposite side of said covered portion, a bath of melted 90 coating metal in said tank and contacting with the cover thereof to exclude air from contact with the upper surface of said bath, means for heating the melted metal in said bath, said heating means being arranged to maintain a higher temperature adjacent the exit opening than that adjacent the entrance opening, and means for progressively feeding articles through said bath from the entrance to the exit opening thereof. 95

4. Galvanizing apparatus, comprising a refractory tank having a cover for the central portion thereof and having entrance and exit openings at opposite ends thereof, electrical 100 heating elements adjacent the outer surface of the wall of said tank for heating a bath of molten metal within said tank, said heating elements being arranged to maintain a higher temperature in said bath adjacent the exit opening thereof than that adjacent the entrance opening thereof, and means for feeding separate articles progressively through said tank from the entrance to the exit opening thereof. 105

5. Galvanizing apparatus, comprising a refractory tank having the top portion thereof closed between its ends, an entrance opening at one end of said tank, a plunger arranged to reciprocate in said tank adjacent said entrance opening to feed separate articles through said tank, said tank having an exit opening at the end thereof opposite said plunger, and electrical heating elements wound about said tank and arranged to generate a greater amount of heat adjacent the exit opening thereof than adjacent the entrance opening thereof. 110

6. Apparatus for coating articles comprising a receptacle having the top thereof closed but having entrance and exit openings, mol- 125

ten coating metal in said receptacle, means for heating said metal to a higher temperature adjacent the exit opening than adjacent the entrance opening, the walls of said receptacle being formed of refractory material and having electrical heating elements connected therewith.

7. Apparatus for galvanizing metal articles comprising a container having a cover, 10 means for heating zinc in said container to a temperature above the melting point of the zinc, the melted zinc in said container being in contact with the cover of said container to exclude air from the surface of said zinc, said 15 heating means being adapted to maintain said zinc at a higher temperature in one portion of said bath than in another, and means for passing the articles to be galvanized through said bath from the cooler to the hot- 20 ter portion thereof.

In testimony whereof I have signed my name to this specification this 12th day of September, A. D. 1928.

ARTHUR O. AUSTIN.

25

30

35

40

45

50

55

60

65